

## UNITED STATES PATENT OFFICE.

TRUMAN S. FULLER, OF SCHENECTADY, NEW YORK, ASSIGNOR TO GENERAL ELECTRIC COMPANY, A CORPORATION OF NEW YORK.

## NICKEL ALLOY.

No Drawing.

Application filed February 16, 1925. Serial No. 9,425.

- This application sets forth an invention comprising a new alloy, and constitutes a continuation in part of my prior application, Ser. No. 699,894, filed March 17, 1924.
- 5 In this prior application, which covers in particular a process of improving the physical properties of certain alloys, I have also described a new alloy or metal composition comprising nickel, copper, aluminum and 10 carbon as constituents.
- I desire in the present application to make claims on an alloy composition constituted largely of nickel and copper which also contains certain correlated proportions 15 of aluminum and carbon as set forth with particularity in the appended claims without restriction to any treatment to which the alloys may be subjected during the course of manufacture.
- 20 An alloy comprising by weight about two-thirds parts of nickel and one-third part of copper and known as Monel metal is used for some purposes because of its non-corrodibility. However, by reason of its only 25 moderate tensile strength and relatively low elastic limit, this alloy is excluded from many industrial uses which require a metal having physical properties approximating the properties of steel.
- 30 I have discovered that by the presence of both aluminum and carbon in definitely related proportions nickel-copper alloys are rendered susceptible to treatment which produces marked improvements in physical 35 properties, particularly in the elasticity of the alloys. The amount of aluminum may vary over several per cent and the amount of carbon over several tenths of one per cent, the aluminum and carbon contents being 40 associated in an inverse ratio with respect to one another as hereinafter more fully explained.
- The advantages of my invention may be 45 best appreciated from the following specific example. An alloy comprising about 60 to 75 parts of nickel, about 25 to 40 parts of copper, about 2.5 parts of aluminum and about 0.16 to 0.17 parts of carbon when forged, or otherwise deformed, below about 50 1000° C. and suitably heat treated has an ultimate tensile strength varying from about 123,000 to 144,000 pounds to the square inch, an elastic limit varying from about 85,000 to 103,000 pounds to the square inch and has 55 a reduction of area at the break varying from about 51 to 58%. The specific physical properties vary somewhat with the conditions of working, heat treating and so forth. Ordinarily Monel metal when subjected to the same conditions and treatment has a materially lower elastic limit and lower tensile strength. The elastic property of a nickel-copper alloy may be improved over 40% when aluminum and carbon are present in properly related proportion. 60
- In carrying out my invention, an alloy of copper and nickel is prepared by any suitable method, for example, by simple fusion of the nickel and the copper in desired proportions. The nickel content may 65 be varied considerably but ordinarily should be as high as 50 per cent, the copper content being increased as the nickel content is decreased. The desired amount of aluminum is stirred into the molten nickel-copper alloy, preferably in an amount less than three per cent. The carbon may be introduced as a high carbon cast iron or other suitable carbon-containing material. Preferably some deoxidizer, such as manganese, 70 also is added to the alloy. If desired the carbon may be introduced as "spiegeleisen" with the manganese. 75
- As already indicated the carbon content 80 preferably should be varied in an inverse measure with the aluminum content. The aluminum content in general may vary from about one-half of one per cent to five per cent. The carbon content may vary from about 0.40 to 0.03 per cent, the higher carbon content being used with the lower aluminum content and vice versa. A preferred 85 alloy contains about 2.5 per cent aluminum and about .16 per cent carbon.
- The preparation and advantages of an 90 alloy embodying my invention may be illustrated by the following specific case. To a molten alloy of about 65 parts nickel and 35 parts copper about 2.5 to 3.5 parts of aluminum are admixed by stirring. About 1.5 95 parts of manganese are stirred into the melt and about 2.5 to 5 parts by weight of high carbon cast iron are added, thereby introducing about 0.1 to 0.2 per cent of carbon 100 into the alloy. 105
- After the carbon has been added about one-tenth of one per cent of magnesium is stirred into the melt as described and claimed in a copending application, Serial No. 699,895, filed by Eric T. Asp on March 110

17, 1924. The addition of magnesium has some effect on the grain of the alloy and renders it more forgeable.

When an alloy thus prepared is forged at temperatures below 1000° C. in accordance with the method claimed in my prior application, Serial No. 699,894, filed March 17, 1924, the remarkable physical properties are developed to the highest degree. For example, the metal may be forged first at about 1000° C. or somewhat lower and preferably finished at about 750° C. or even at a lower temperature.

After forging the alloy is treated by holding the same at 500° to 700° C. for about six hours and then cooling slowly, that is bringing the alloy to room temperature in several hours.

The wrought metal thus produced has physical properties comparable to a high grade of steel while still retaining the corrosion-resisting properties of ordinary copper-nickel alloys. It is particularly useful for industrial applications requiring a combination of both properties, for example, turbine buckets and marine devices.

What I claim as new and desire to secure by Letters Patent of the United States, is:—

1. An alloy consisting mainly of nickel and copper and containing from about one-half to five per cent aluminum and from about 0.40 to 0.03 per cent carbon, the higher aluminum content in a given alloy being associated with the lower carbon content and vice versa.

2. A wrought alloy comprising at least about 50 per cent nickel containing about one-half to five per cent of aluminum and from about 0.40 to 0.03 per cent of carbon, the balance of the alloy being predominantly copper, said alloy being characterized by a tensile strength in excess of about 100,000 pounds per square inch, an elastic limit in excess of 80,000 pounds to the square inch and a high ductility.

3. An alloy comprising by weight of about two-thirds nickel and one-third copper and containing about 2.5 per cent aluminum and about 0.16 per cent carbon, and

having when forged an elasticity equal to 50 high-grade steel.

4. An alloy comprising about 60 parts nickel, about 35 parts copper, about 2.5 parts aluminum, about 0.16 parts carbon, about 1.5 parts manganese and about 2.5 parts 55 iron, said alloy being capable of developing by mechanical work and heat treatment a tensile strength as high as about 120,000 pounds per square inch and an elastic limit approximating 100,000 pounds per square 60 inch.

5. An alloy consisting mainly of nickel and copper, the nickel being in excess of the copper and containing about one-half to five per cent aluminum and about .40 to .03 65 per cent carbon, the higher aluminum content in a given alloy being associated with the lower carbon content and vice versa.

6. An alloy comprising 60 to 75 parts nickel and 25 to 40 parts copper, and containing one-half to five per cent aluminum and .40 to .03 per cent carbon, the higher 70 aluminum content in a given alloy being associated with the lower carbon content and vice versa.

7. An alloy containing nickel, copper, aluminum and carbon wherein the nickel content is in excess of 50 per cent, the content of aluminum is from one-half to five per cent, the carbon content from .40 to .03 per cent, 80 the predominating metal of the remaining content being copper, the higher aluminum content in a given alloy being associated with the lower carbon content and vice versa.

8. An alloy containing nickel, copper, aluminum and carbon, wherein the nickel content is not substantially less than 50 per cent, the content of aluminum is from one-half to five per cent, the carbon content 90 from .40 to .03 per cent, the predominating metal of the remaining content being copper, the higher aluminum content in a given alloy being associated with the lower carbon content and vice versa.

In witness whereof, I have hereunto set my hand this 14th day of February, 1925.

TRUMAN S. FULLER.

17, 1924. The addition of magnesium has some effect on the grain of the alloy and renders it more forgeable.

When an alloy thus prepared is forged at temperatures below 1000° C. in accordance with the method claimed in my prior application, Serial No. 699,894, filed March 17, 1924, the remarkable physical properties are developed to the highest degree. For example, the metal may be forged first at about 1000° C. or somewhat lower and preferably finished at about 750° C. or even at a lower temperature.

After forging the alloy is treated by holding the same at 500° to 700° C. for about six hours and then cooling slowly, that is bringing the alloy to room temperature in several hours.

The wrought metal thus produced has physical properties comparable to a high grade of steel while still retaining the corrosion-resisting properties of ordinary copper-nickel alloys. It is particularly useful for industrial applications requiring a combination of both properties, for example, turbine buckets and marine devices.

What I claim as new and desire to secure by Letters Patent of the United States, is:—

1. An alloy consisting mainly of nickel and copper and containing from about one-half to five per cent aluminum and from about 0.40 to 0.03 per cent carbon, the higher aluminum content in a given alloy being associated with the lower carbon content and vice versa.

2. A wrought alloy comprising at least about 50 per cent nickel containing about one-half to five per cent of aluminum and from about 0.40 to 0.03 per cent of carbon, the balance of the alloy being predominantly copper, said alloy being characterized by a tensile strength in excess of about 100,000 pounds per square inch, an elastic limit in excess of 80,000 pounds to the square inch and a high ductility.

3. An alloy comprising by weight of about two-thirds nickel and one-third copper and containing about 2.5 per cent aluminum and about 0.16 per cent carbon, and

having when forged an elasticity equal to 50 high grade steel.

4. An alloy comprising about 60 parts nickel, about 35 parts copper, about 2.5 parts aluminum, about 0.16 parts carbon, about 1.5 parts manganese and about 2.5 parts 55 iron, said alloy being capable of developing by mechanical work and heat treatment a tensile strength as high as about 120,000 pounds per square inch and an elastic limit approximating 100,000 pounds per square 60 inch.

5. An alloy consisting mainly of nickel and copper, the nickel being in excess of the copper and containing about one-half to five per cent aluminum and about .40 to .03 65 per cent carbon, the higher aluminum content in a given alloy being associated with the lower carbon content and vice versa.

6. An alloy comprising 60 to 75 parts nickel and 25 to 40 parts copper, and containing one-half to five per cent aluminum and .40 to .03 per cent carbon, the higher aluminum content in a given alloy being associated with the lower carbon content and vice versa.

7. An alloy containing nickel, copper, aluminum and carbon wherein the nickel content is in excess of 50 per cent, the content of aluminum is from one-half to five per cent, the carbon content from .40 to .03 per cent, the predominating metal of the remaining content being copper, the higher aluminum content in a given alloy being associated with the lower carbon content and vice versa.

8. An alloy containing nickel, copper, aluminum and carbon, wherein the nickel content is not substantially less than 50 per cent, the content of aluminum is from one-half to five per cent, the carbon content 90 from .40 to .03 per cent, the predominating metal of the remaining content being copper, the higher aluminum content in a given alloy being associated with the lower carbon content and vice versa.

In witness whereof, I have hereunto set my hand this 14th day of February, 1925.

TRUMAN S. FULLER.

#### Certificate of Correction.

Patent No. 1,623,948.

TRUMAN S. FULLER.

Granted April 5, 1927, to

It is hereby certified that error appears in the printed specification of the above-numbered patent requiring correction as follows: Page 1, line 59, for the word "Ordinarily" read *Ordinary*; and that the said Letters Patent should be read with this correction therein that the same may conform to the record of the case in the Patent Office.

Signed and sealed this 24th day of May, A. D. 1927.

[SEAL.]

M. J. MOORE,  
Acting Commissioner of Patents.

**Certificate of Correction.**

Patent No. 1,623,948.

Granted April 5, 1927, to

TRUMAN S. FULLER.

It is hereby certified that error appears in the printed specification of the above-numbered patent requiring correction as follows: Page 1, line 59, for the word "Ordinarily" read *Ordinary*; and that the said Letters Patent should be read with this correction therein that the same may conform to the record of the case in the Patent Office.

Signed and sealed this 24th day of May, A. D. 1927.

[**SEAL.**]

M. J. MOORE,  
*Acting Commissioner of Patents.*